

## UNITED STATES PATENT OFFICE

2,666,745

## CORROSION PREVENTING AGENT

Leo V. Mullen, Jr., Clifton, and James M. Boyle,  
Bayonne, N. J., assignors to Standard Oil De-  
velopment Company, a corporation of Delaware

No Drawing. Application December 1, 1950,  
Serial No. 198,763

16 Claims. (Cl. 252—47)

1

The present invention relates to the improvement of hydrocarbon oil products, especially those derived from petroleum sources, and more particularly to the preparation of improved mineral lubricating oil compositions by the incorporation therein of a new class of additives which impart improved properties to such oils and compositions containing them.

In the development of petroleum lubricating oils the trend has been to use more and more efficient refining methods in order to reduce the tendency of the oils to form carbon and deposits of solid matter or sludge. While such highly refined oils possess many advantages, their resistance to oxidation, particularly under conditions of severe service, is generally decreased and they are more prone to form soluble acidic oxidation products which are corrosive. They are generally less effective than the untreated oils in protecting the metal surfaces which they contact against rusting and corrosion due to oxygen and moisture. Although generally superior to lightly refined oils they may deposit films of "varnish" on hot metal surfaces, such as the pistons of internal combustion engines, under very severe engine operating conditions.

In accordance with the present invention a new class of substances has been discovered which when added to refined lubricating oils and other petroleum oil products in small proportions substantially reduce the tendency of such oils to corrode metal surfaces and which are particularly effective in inhibiting the corrosion of copper-lead and cadmium-silver bearings.

The new class of materials which have been found to possess the stabilizing and detergent qualities described above are reaction products obtained by first reacting an unsaturated di-aliphatic hydrocarbon - substituted cyanamide with a primary or secondary aliphatic or cyclo-aliphatic amine and subsequently sulfurizing the product thus formed with elemental sulfur, or other agents which introduce sulfur into the unsaturated aliphatic groups, until from 10 to 30% of sulfur has been combined therewith. In the reaction between the cyanamide and the amine the reactants are employed in substantially equimolar amounts and the reaction normally takes place within the temperature range of about 100 to about 250° C. The reaction is substantially complete within a period of 1 to 10 hours. In the sulfurizing reaction flowers of sulfur are usually employed and the reaction takes place at 80-150° C. within a period of about 1 to 4 hours.

2

It is possible that the above described reaction between a dialkyl cyanamide and an amine takes place in accordance with the equation:



10 where R and R' are aliphatic hydrocarbon groups of the cyanamide, at least one of which is unsaturated and R'' is the hydrocarbon group of the amine. The above is merely a suggested equation, since the exact constitution of the reaction product is not known with certainty.

15 The unsaturated disubstituted cyanamide employed in the above described reaction may be any cyanamide containing one or more double or triple bonds in at least one aliphatic group, and such aliphatic groups may contain from 1 to 30 carbon atoms each. The aliphatic groups may be straight or branched and may contain substituent halogen atoms. Examples of suitable disubstituted cyanamides are diallyl cyanamide, methyl allyl cyanamide, dioleyl cyanamide, dili-  
20 noleyl cyanamide, di-4-propenyl octyl cyanamide, and di-n-octadecenyl cyanamide.

25 The aliphatic or cycloaliphatic amines which may be employed in the above reaction may be any primary or secondary, saturated or unsaturated amine containing from 1 to 30 carbon atoms. Examples of such amines are methylamine, ethylamine, isopropylamine, n-hexylamine, n-octylamine, 2-ethylhexylamine, "Lorol" amine (a derivative of coconut oil acids consisting of a mixture of C<sub>10</sub> to C<sub>18</sub> primary aliphatic amines), "Armeen 14D" (a composition consisting chiefly of n-tetradecylamine with small quantities of n-dodecylamine, n-hexadecylamine, and an octadecylamine), dimethylamine, diethylamine, 40 dicetylamine, cyclohexylamine, and dicyclohexylamine.

45 The preferred compositions of the present invention are obtained by reacting a disubstituted cyanamide with an amine in accordance with the method described above and sulfurizing the product with elemental sulfur. However, other products of similar nature and having corrosion inhibiting and antioxidant properties may be prepared by reacting the cyanamide-amine product with a sulfur chloride or bromide to introduce both sulfur and a halogen into the product, and further reacting this product with an alkali metal mercaptide, xanthate, thiocarbamate, thiophosphate, or phenate, whereby the halogen 50 is removed as an alkali metal halide and the

mercaptide or other group is joined to the molecule.

The quantity of the additives of the present invention which is most advantageously blended in mineral lubricating oils or other petroleum hydrocarbon products will depend upon the property of the additive which it is most desired to exploit. When employed for detergent and sludge dispersing properties, the quantity most suitable will generally vary from 1 to 5% by weight. For merely inhibiting bearing corrosion and generally when employed as an antioxidant the quantity most desired will be from 0.05 to 2%, although quantities as great as 5% may on occasion be used. For commercial purposes, it is convenient to prepare concentrated oil solutions in which the amount of additive in the composition ranges from 25 to 50% by weight and to transport and store them in such form. In preparing a lubricating oil composition for use as a crankcase lubricant, the concentrate will be prepared from a lubricating base oil and will be blended with additional quantities of the base oil as and when required.

The preparation and testing of an example of the new additives of the present invention are illustrated by the examples to be described in detail below, but it is to be understood that this preparation is illustrative only and is not intended to limit the scope of the invention in any manner.

*Example 1.—Preparation of additive*

(a) 20 g. (0.16 mol) of diallyl cyanamide was added dropwise to 37.5 g. (0.17 mol) of molten "Armeen 14D,"<sup>1</sup> and the resulting solution was refluxed at 210° C. for 6 hours. The reaction mixture was cooled and filtered, and the resulting orange-red oily liquid was found to have the following composition:

|          | Per cent |
|----------|----------|
| Nitrogen | 10.91    |
| Carbon   | 75.74    |
| Hydrogen | 12.65    |

(b) To 32 g. of the reaction product prepared above was added 12 g. of flowers of sulfur. The resulting mixture was heated at 100° C. for 3 hours and the product was filtered through "Hi-Flo" (a filter-aid). The product had the following composition:

|          | Per cent |
|----------|----------|
| Sulfur   | 19.78    |
| Nitrogen | 9.28     |

*Example 2.—Laboratory bearing corrosion test*

A blend containing 0.25% by weight of the product of Example 1 in a paraffinic type mineral lubricating oil of SAE 20 grade and a sample of the unblended base oil were submitted to a corrosion test designed to measure the effectiveness of the product in inhibiting the corrosiveness of a typical mineral lubricating oil towards the surfaces of copper-lead bearings. The test was conducted as follows: 500 cc. of the oil was placed in a glass oxidation tube (13 inches long and 2½ inches in diameter) fitted at the bottom with a ¼ inch air inlet tube perforated to facilitate air distribution. The oxidation tube was then immersed in a heating bath so that the oil tempera-

ture was maintained at 325° F. during the test. Two quarter sections of automotive bearings of copper-lead alloy of known weight having a total area of 25 sq. cm. were attached to opposite sides of a stainless steel rod which was then immersed in the test oil and rotated at 600 R. P. M., thus providing sufficient agitation of the sample during the test. Air was then blown through the oil at the rate of 2 cu. ft. per hour. At the end of each 4-hour period the bearings were removed, washed with naphtha, and weighed to determine the amount of loss by corrosion. The bearings were then repolished (to increase the severity of the test), reweighed, and then subjected to the test for additional 4-hour periods in like manner. The results are given in the following table as "corrosion life," which indicates the number of hours required for the bearings to lose 100 mg. in weight, determined by interpolation of the data obtained in the various periods.

| Oil or Oil Blend                      | Bearing Corrosion Life (Hrs.) |
|---------------------------------------|-------------------------------|
| Base oil                              | 19                            |
| Base oil + 0.25% product of Example 1 | 25                            |

*Example 3.—Lauson engine test*

A blend containing 1% by weight of the product of Example 1 in a solvent extracted naphthenic oil of 60 seconds Saybolt viscosity at 210° F. and a sample of the unblended base oil were employed as the crankcase lubricant in tests with a Lauson engine operating at 295° F. jacket temperature and 300° F. oil temperature, 1800 R. P. M. speed, and 1.5 indicated kilowatt load, the tests being conducted for 25 hours each. The loss in weight of the copper-lead bearing was determined in each case. The results of the tests are as follows:

| Lubricant                          | Bearing Weight Loss (gm./bearing) |
|------------------------------------|-----------------------------------|
| Base oil                           | 0.039                             |
| Base oil + 1% product of Example 1 | 0.012                             |

The products of the present invention may be employed not only in ordinary hydrocarbon lubricating oils but also in the "heavy duty" type of lubricating oils which have been compounded with such detergent type additives as metal soaps, metal petroleum sulfonates, metal phenates, metal alcoholates, metal alkyl phenol sulfides, metal organo phosphates, phosphites, thiophosphates, and thiophosphites, metal xanthates and thioxanthates, metal thiocarbamates, and the like. Other types of additives, such as phenols and phenol sulfides, may also be present.

The lubricating oil base stock used in the compositions of this invention may be straight mineral lubricating oils or distillates derived from paraffinic, naphthenic, asphaltic or mixed base crudes, or, if desired, various blended oils may be employed as well as residuals, particularly those from which asphaltic constituents have been carefully removed. The oils may be refined by conventional methods using acid, alkali and/or clay or other agents such as aluminum chloride, or they may be extracted oils produced by solvent extraction with solvents such as phenol, sulfur dioxide, etc. Hydrogenated oils or white oils may be employed as well.

<sup>1</sup> Armeen 14D has the following composition:

|                   | Per cent |
|-------------------|----------|
| n-Dodecylamine    | 4        |
| n-Tetradecylamine | 90       |
| n-Hexadecylamine  | 4        |
| Octadecylamine    | 2        |

as synthetic oils resembling petroleum oils, prepared, for example, by the polymerization of olefins or by the reaction of oxides of carbon with hydrogen or by the hydrogenation of coal or its products.

For the best results the base stock chosen should normally be an oil which with the new additive present gives the optimum performance in the service contemplated. However, since one advantage of the additives is that their use also makes feasible the employment of less satisfactory mineral oils, no strict rule can be laid down for the choice of the base stock. The additives are normally sufficiently soluble in the base stock, but in some cases auxiliary solvent agents may be used. The lubricating oils will usually range from about 40 to 150 seconds (Saybolt) viscosity at 210° F. The viscosity index may range from 0 to 100 or even higher.

Other agents than those which have been mentioned may be present in the oil composition, such as dyes, pour point depressants, heat thickened fatty oils, sulfurized fatty oils, sludge dispersers, antioxidants, thickeners, viscosity index improvers, oiliness agents, resins, rubber, olefin polymers, and the like.

Assisting agents which are particularly desirable as plasticizers and defoamers are the higher alcohols having preferably 8-20 carbon atoms, e. g., octyl alcohol, lauryl alcohol, stearyl alcohol, and the like.

In addition to being employed in lubricants, the additives of the present invention may also be used in other hydrocarbon oil products such as motor fuels, heating oils, hydraulic fluids, torque converter fluids, cutting oils, flushing oils, turbine oils, transformer oils, industrial oils, process oils, and the like, and generally as antioxidants in mineral oil products. They may also be used in gear lubricants, greases and other products containing mineral oils as ingredients.

What is claimed is:

1. A hydrocarbon oil containing a corrosion inhibiting amount of a product obtained by reacting together substantially equimolar amounts of a dialiphatic hydrocarbon substituted cyanamide, containing 1 to 30 carbon atoms in each aliphatic group and containing at least one unsaturated grouping in at least one of such aliphatic groups, and an amine selected from the group consisting of primary and secondary aliphatic and cycloaliphatic amines containing 1 to 30 carbon atoms at a temperature of 100-250° C., and sulfurizing such reaction product by reacting the same with elemental sulfur until 10 to 30% of sulfur is combined therewith.

2. A composition according to claim 1 in which the hydrocarbon oil is a mineral lubricating oil.

3. A composition according to claim 2 in which the disubstituted cyanamide contains one olefinic grouping in each aliphatic group and in which the amine is a primary aliphatic amine.

4. A composition according to claim 3 in which the disubstituted cyanamide is diallyl cyanamide.

5. A composition according to claim 4 in which the amine is essentially a primary aliphatic amine containing 12 to 18 carbon atoms.

6. A composition according to claim 5 containing approximately 20% of sulfur.

7. A composition consisting essentially of a mineral lubricating oil and the additive as defined in claim 1, the amount of said additive in the composition being 25 to 50% by weight.

8. A composition consisting essentially of a mineral lubricating oil and an additive as de-

fined in claim 6, the amount of said additive in the composition being 25 to 50% by weight.

9. As a new composition of matter a product obtained by reacting together substantially equimolar amounts of a dialiphatic hydrocarbon-substituted cyanamide, containing 1 to 30 carbon atoms in each aliphatic group and containing at least one unsaturated grouping in at least one of such aliphatic groups, and an amine selected from the group consisting of primary and secondary aliphatic and cycloaliphatic amines containing 1 to 30 carbon atoms at a temperature of 100-250° C., and sulfurizing such reaction product by reacting the same with elemental sulfur until 10 to 30% of sulfur is combined therewith.

10. A composition according to claim 9 in which the disubstituted cyanamide contains one olefinic group in each aliphatic group and in which the amine is a primary aliphatic amine.

11. A composition according to claim 9 in which the disubstituted cyanamide is diallyl cyanamide and in which the amine is a primary aliphatic amine containing 12 to 18 carbon atoms.

12. A composition according to claim 11 containing approximately 20% of sulfur.

13. The process which comprises reacting together substantially equimolar amounts of an unsaturated, dialiphatic hydrocarbon-substituted cyanamide containing 1 to 30 carbon atoms in each aliphatic group and an amine selected from the group consisting of primary and secondary aliphatic and cycloaliphatic amines containing 1 to 30 carbon atoms at a temperature of 100-250° C., and sulfurizing such reaction product by reacting the same with elemental sulfur until 10 to 30% of sulfur is combined therewith.

14. A process according to claim 13 in which the disubstituted cyanamide contains one olefinic group in each aliphatic group, in which the amine is a primary aliphatic amine, and in which the sulfurizing step takes place at a temperature of 80 to 150° F.

15. A process according to claim 14 in which the disubstituted cyanamide is diallyl cyanamide, in which the amine is a primary aliphatic amine containing 12 to 18 carbon atoms, and in which the sulfurizing step is continued until 20% by weight of sulfur is combined with the reaction product.

16. The process which comprises refluxing a mixture of substantially equimolar amounts of diallyl cyanamide and a mixture of primary aliphatic amines containing 12 to 18 carbon atoms at a temperature of about 210° C. for a period of about 6 hours, and heating the resulting reaction product with elemental sulfur at about 100° C. for a period of about 3 hours.

LEO V. MULLEN, JR.  
JAMES M. BOYLE.

References Cited in the file of this patent

UNITED STATES PATENTS

| Number    | Name                   | Date          |
|-----------|------------------------|---------------|
| 1,766,755 | Lecher et al. -----    | June 24, 1930 |
| 2,209,464 | Loane et al. -----     | July 30, 1940 |
| 2,263,562 | Bigelow et al. -----   | Nov. 25, 1941 |
| 2,325,586 | Bolton et al. -----    | Aug. 3, 1943  |
| 2,425,341 | Paden et al. -----     | Aug. 12, 1947 |
| 2,542,982 | Bartleson et al. ----- | Feb. 27, 1951 |

OTHER REFERENCES

Zeile et al.: Zeitschrift Physiol. Chem., vol. 75 256 (1938), pp. 131-132.